

## UNITED STATES PATENT OFFICE.

HUGH H. HANSARD, OF MONTREAL, QUEBEC, CANADA.

## FUEL BRIQUETTE AND METHOD OF MAKING SAME.

No Drawing.

Application filed June 23, 1924. Serial No. 721,939.

This invention relates broadly to fuel briquettes and to the method of making same, and relates more particularly to briquettes made from coal.

5 An object of the invention is to provide a briquette which will burn with little or no smoke and without disintegration or adhering to adjoining briquettes, and which will further be sufficiently porous to ignite readily and burn at a desirable rate.

Another object is to provide a briquette sufficiently hard to withstand transportation and much handling, and also exposure to weather without appreciable disintegration 10 and without undue absorption of moisture.

Still another object is to provide a briquette having an ash content as low as possible and in the case of briquettes made from coal with a clinkering tendency, a substantial 15 freedom from clinkering.

A further object is to provide a process of manufacturing briquettes which will enable fulfilment of the foregoing objects.

Still another object is to provide a process 20 of manufacturing briquettes which may be carried out inexpensively and economically.

An additional object is to provide a process 25 which, with suitable variations, is applicable to the briquetting of any grade of coal, and particularly to certain grades of coal which are not generally available for fuel purposes, to produce therefrom high grade fuel briquettes capable of replacing 30 any of the grades of coal ordinarily used as fuel.

Various other objects and advantages may be ascertained from the following description.

40 The problem of briquetting materials, particularly coal, for use as fuel is one which has received a great deal of attention in recent years. Rapidly approaching exhaustion of the higher grades of coal makes it 45 necessary to devise means for employing the lower grades of coal and at the same time with efficiency equal to or greater than that obtained with the higher grades, so as to enable the lower grades of coal to be used under the conditions which have led to and 50 arisen from the extensive use of the higher grades of coal.

The principal difference between the 55 various grades of coal is a matter of carbonization and accompanying this is the question of ash content. Coals, such as an-

thracite, are highly carbonized and contain only a small percentage of volatiles so that they are clean to handle and burn practically smokelessly, making them particularly 60 fitted for domestic use and for commercial use in large centers of population where smoke must be avoided as much as possible. Some of these coals have the disadvantage of high ash content. Other grades of coal, 65 while less carbonized, have greater fuel value but because of a higher percentage of volatiles and the relatively lower carbonization their combustion is accompanied by the emission of much smoke so that they are unsuitable for domestic and for many commercial 70 purposes. Still other grades of coal, commonly included under the term lignites, are but little carbonized and contain a relatively large percentage of volatiles, also considerable moisture, so that they are unsuitable for most commercial uses unless burned in specially constructed furnaces or subjected to special treatment to overcome or offset their inherent disadvantages. 75

The general method of briquetting coal is to incorporate the pulverized coal with a hydrocarbon binder, such as pitch or asphalt, and then to press the mixture into briquettes. Experience has shown that hydrocarbon 80 binders which mix readily with the powdered coal produce briquettes which are comparatively soft and in which the binder has a low melting point, so that the briquette disintegrates with transportation or handling and 85 also during combustion with the additional disadvantage of adhering to adjoining briquettes. High melting point binders are difficult to incorporate with the powdered coal and as a result an unduly large proportion 90 of binder must be used. The briquettes, while hard enough to withstand transportation and handling and to avoid disintegration during combustion, are so dense as to be difficult to ignite and slow burning. Also the 95 expense of their production is so great as to seriously limit their use.

According to the present invention a briquette may be produced having requisite hardness to avoid disintegration in handling 100 or combustion and which further will not adhere to adjoining briquettes when heated. Such a briquette may be made inexpensively from any grade of coal and if desired the ash content and clinkering elements of the 105 coal may be wholly or largely removed, also the degree of carbonization may be increased 110

and the density varied as necessary to obtain any desired speed of ignition or combustion. The binder as it appears in the finished briquette has a high melting point and moreover is very intimately associated with the particles of coal and in amount sufficient only for binding purpose, so that there is no excess of binder to fill the pores of the briquette rendering the same difficultly combustible. According to the process of manufacture valuable by-products are obtained, the sale of which will substantially cover the cost of briquetting.

The process of briquetting briefly described is as follows: Coal is very finely ground or otherwise pulverized so as to pass through, for example, a 200-mesh screen, although the particles of coal may be either larger or smaller than thus indicated. This pulverized coal if of a quality suitable for immediate briquetting is then mixed with a predetermined amount of a liquid hydrocarbon binder, such as crude oil, preferably that having an asphalt base, or with coal tar or any other suitable hydrocarbon binder. An intimate and thorough mixing of the coal and binder is enabled by the use of a binder suitably fluid in its natural state or rendered suitably fluid by the addition of diluents. The mixing is effected in any well known manner, as by means of a ball mill, and continued until, as nearly as commercially possible, every particle of the pulverized coal has received a film or coating of the binding material. The mixture is then heated with exclusion of air to drive off the volatiles of the binder and the coal itself and also the low boiling portions of the binder, with the result that there remains a mass of coal particles each having a very thin film or coating of high melting binding material. The amount of binding material originally mixed with the coal is gauged according to the nature of the binding material and the temperature at which it will be heated, which temperature is determined partly by the nature of the coal, so that after the heating a predetermined percentage of binder of predetermined melting point will remain. In this way the use of binding material in excess of that actually required for binding purposes may be avoided. The heat treatment also serves to effect a carbonizing action in the coal. After completion of the heat treatment the coated coal particles are pressed in any suitable way into briquettes, which are then ready for use or which may be suitably aged or cured by retention in storage. Owing to the evaporation of the low boiling constituents of the binder and of the volatiles of the coal and binder, it will be readily seen that as only the high boiling constituents remain, requisite hardness to withstand disintegration during handling and combustion will result. The physi-

cal hardness of the briquette and the porosity thereof depend of course to a considerable extent upon the pressure employed in briquetting. Nevertheless, even when using high briquetting pressures the finished briquette will be found more porous and therefore more readily combustible than is ordinarily the case owing to the use of the minimum amount of binder which does not fill the tiny voids between the particles of coal. The volatiles and low boiling material driven off during the heat treatment may be recovered and their value will largely compensate for, or even more than compensate for, the entire cost of treatment and briquetting of the coal, so that briquettes of superior quality may be sold at comparatively low prices. The heating step which causes carbonization of the coal as well as expulsion of volatiles will enable coal, such as bituminous coal or lignites, to be converted into briquettes having the combustion characteristics of anthracite coal or anthracite briquettes.

Where the coal dealt with has an undesirable high ash content the grinding may be sufficiently fine to effect an appreciable or substantially complete mechanical separation of the carbonaceous particles and the ash particles. This powder may then be wet with water and subsequently mixed with the oily binding material. The oily hydrocarbon binder has greater affinity for the carbon particles than for the ash particles with the result that an effective separation of carbon and ash may be effected to eliminate the ash, as fully described in United States Patent No. 1,420,165, granted the 20th June 1922.

If has furthermore been discovered that when dealing with coals containing a sufficient percentage of readily separable bitumen no additional binder is required but merely the addition of a diluent to co-operate with the heat treatment in extracting the bitumen from the coal. During the heat treatment and by means of an oily diluent or solvent, bitumen is extracted from the coal and serves as a binder. In such a case substantially all the solvent or diluent may be distilled off and in addition a considerable amount of volatiles contained in the coal. Also, when dealing with coals having available binding material less than required for briquetting purposes, only that amount of binder necessary to make up the deficiency need be added.

The heat treatment may be effected in any suitable furnace or retort, preferably one provided with means for rabbling the mixture and composed of iron or other material having a catalytic action in the distillation of volatiles from the binder and coal. The retort used is preferably one of considerable length in which the material may pass slow-

ly from a cool zone with gradually increasing temperature to a hot zone at the discharge end.

In order that a better understanding of the invention may be obtained, the following specific example is given, but it will be understood that the invention is in no way limited to the details of this example.

10 *Example I.*

The materials used are coal analyzing approximately:

|              | Per cent. |
|--------------|-----------|
| Moisture     | 0.80      |
| 15 Volatile  | 26.00     |
| Fixed carbon | 52.00     |
| Ash          | 20.00     |
| Sulphur      | 1.20      |

20 and a heavy oil, such as Mexican oil having an asphalt base and which will lose approximately 50% of its weight at or slightly under 650° F.

The coal is pulverized so that it will all 25 pass through a 200-mesh screen. This coal is mixed with the oil in the proportion of 12 to 20 parts of oil to 98 parts of coal by weight. The mixing is effected very thoroughly by means of a ball-mill or the like and continued until substantially every particle of 30 coal has acquired a coating or enveloping film of oil. The mixture is then transferred to a suitable retort, for example, such as made by The American Continuous Retort 35 Company for treatment of oil shales. The mixture is passed through the retort, the temperature of which gradually increases to approximately 650° F. at the discharge end. During this retorting volatiles are driven off 40 and may be collected. These volatiles represent about half the weight of the oil and about 4 parts by weight of the coal. Starting with 12 parts of oil and 98 parts of coal by weight the mixture discharged from the 45 retort will have a composition of 6 parts of binding material having a distillation temperature of 650° F. or over, and 94 parts of coal. The mixture is then briquetted in any suitable press and the resulting briquette 50 when completely cooled will be found sufficiently hard to stand transportation and handling without disintegration. Owing to the distribution of the binder through the pulverized coal when in fluid condition and the subsequent abstraction of volatiles, there 55 is left on each particle of coal a thin coating of binder sufficient to cause the particles to adhere when pressed and yet not sufficient to close the voids between particles. The 60 briquette, while sufficiently tough to withstand transportation and handling, also possesses the porosity necessary for satisfactory combustion and to avoid disintegration of the briquette by gases generated within the 65 same. The binder in a freshly made bri-

quette has a melting point of 300° F. to 375° F. or over and with ageing this melting point gradually rises. When the briquettes are placed in a fire the first effect of heat is to further raise the melting point of the 70 binder and drive off as gas some of the constituents. The porous nature of the briquette permits the escape of these gases without disintegration of the briquette and the unburned binder becomes more and more 75 carbonized. The driving off of volatiles during the manufacture of the briquette removes a large part of the constituents of both the binder and the coal which cause 80 smoking. This effect is further increased by the carbonization which takes place, with the result that the briquettes produced will burn with little or no smoke and are comparable in this respect and also in their speed of burning with anthracite coal.

If the pulverized coal is mixed with water before addition of the oil it will be found that the oil, which has a greater affinity for the carbon particles than for the ash particles, will adhere to the carbon particles 90 to a greater extent than to the ash particles, with the result that the ash or non-carbon particles may be washed out. Using coal of the analysis given and thus purified a freshly made briquette will analyze approximately: 95

|                  |                  |
|------------------|------------------|
| Moisture         | nil              |
| Volatile         | 26%              |
| Fixed carbon     | 73%              |
| Sulphur          | 1%               |
| Ash, trace up to | 1/2%             |
| B. t. u.         | 14,500 to 15,500 |

It will be understood that it is impossible to lay down any proportion of liquid binding material and coal, as the proportion depends upon the nature of the coal and particularly upon the amount of volatiles and the amount of available binding material in the coal, also upon the amount of ash and whether the same is to be removed or not. It may be stated, however, that in the finished briquette there should be from 6 to 10 parts by weight of binder having a melting point of 300° F. or over and serving to agglomerate 94 to 90 parts of coal. It will also be obvious that the proportion of oil mixed with the coal will, to some extent, be governed by the nature of the oil and its distillation range.

While it has been previously stated that bituminous coals and lignites will be carbonized, it must be understood that this does not refer to complete carbonization such as would render the material incapable of combustion under ordinary conditions, but merely to an increased degree of carbonization. It has also been stated that with certain grades of coal containing a comparatively large amount of soluble material ca-

pable of use as a binder, only a solvent for this material need be used, but it must not be concluded that the abstraction of binding material from the coal is confined to the use of merely solvent liquids. When dealing with bituminous coals or lignites a certain amount of binding material is available in the coal and will be obtained by the distillation step regardless of whether the liquid added is purely a solvent or is diluted with binding material. Therefore, the amount of liquid binding material used may be varied according to the nature of the coal. On the other hand where the coal will provide sufficient binding material the solvent liquid added may be in itself incapable of acting as a binder or of being resolved into a binding material. It will therefore be understood that the invention is not confined to the addition of the amounts of binding material stated to be found in the completed briquette, nor to any particular temperature or duration of distillation treatment, or to carbonization or any particular degree of carbonization of the carbonaceous matter, but relates to any means by which a small amount of high melting binding material may be intimately incorporated with carbonaceous material, the amount of such binder being usually less than could be mechanically incorporated to produce a satisfactory coating of the carbonaceous particles without the presence of sufficient binder to fill the interstices of the finished briquette.

While in the foregoing example the melting temperature of the binder has been given as 300° to 375° F. and the distillation temperature thereof as 650° F. or higher, it must be understood that the invention is not limited to these temperatures as satisfactory briquettes may be made using binders which melt considerably below 300° F. and which distil considerably below 650° F. Further, the invention, as regards the manner of incorporating the binder and coal, is not subject to any temperature limitations except those of practicability.

Instead of immediately briquetting the mixture of binder and finely pulverized coal, this mixture may be itself used as a binding material for a further amount of coal. When operating in this manner it is preferable to increase the proportion of binding material to the finely pulverized coal, and to have the additional coal in relatively coarse particles. The following example will serve to illustrate.

*Example II.*

A mixture of pulverized coal, 200-mesh or finer, containing after retorting 82½% coal and 17½% binder, by weight, is mixed with from twice to four times its weight of granulated coal which will pass through, say, a 20-mesh screen. After thorough mixing the

mass is briquetted without further retorting. The resulting briquette is of good quality and may be produced more cheaply than one made entirely from finely pulverized coal and contains a very low percentage of binding material without appreciable sacrifice of the desirable qualities heretofore enumerated. In fact, such a briquette is more porous and therefore burns more rapidly than one made of finely pulverized coal.

As a variation, the mixture of finely pulverized coal and oil may be combined with the coarser coal before retorting. Also, if it is desired to omit the retorting step altogether this manner of mixing may be resorted to for the purpose of obtaining a uniform and intimate mixture of coal and a relatively very small amount of binder. It will be understood that the invention is not limited to the proportions of the binder and finely pulverized coal used to make what may be termed a dry binder for the coarse coal, nor is it limited to the proportions of dry binder and coarse coal.

Having thus described my invention, what I claim is:—

1. A process of making fuel briquettes which consists in mixing pulverized coal and a liquid hydrocarbon, heating the mixture to drive off the volatile and low boiling constituents of the liquid hydrocarbon, and briquetting the resulting mass which consists of pulverized coal and the high boiling residue of the liquid hydrocarbon.

2. A process of making fuel briquettes which consists in mixing pulverized coal with a liquid hydrocarbon, heating the mixture to drive off those constituents thereof which distil at 650° F. or under, and briquetting the remaining mass.

3. A process of making fuel briquettes which consists in mixing pulverized coal and liquid hydrocarbon in proportion to produce eventually from 6% to 10% by weight of hydrocarbon binder having a melting point of 300° F. or over, heating the mixture to separate constituents which distil off below 650° F., and briquetting the resulting mass.

4. A process of making fuel briquettes which comprises coating particles of pulverized coal with a very thin layer of high melting hydrocarbon binder by first coating the particles with the binding material in solution and then heating the coated particles to drive off the solvent, and finally briquetting the coated particles.

5. A process of making fuel briquettes which comprises mixing the finely powdered coal with a liquid hydrocarbon binding material, heating the mixture to drive off volatiles and low boiling constituents of the binding material and to leave as a thin coating on the individual particles of coal a residue having a high melting point, the

total amount of binder being materially less than the least amount of binder of the same melting point that could be directly coated on the particles, and briquetting the coated particles.

6. A process of making fuel briquettes which comprises pulverizing coal to such degree of fineness that a substantial mechanical separation of carbonaceous and non-carbonaceous particles is effected, mixing the powder with water, treating the wet mass with a liquid hydrocarbon binding material which, by its greater affinity for the carbonaceous particles than for the non-carbonaceous particles, will effect a separation of the particles in water, washing out the non-carbonaceous particles, drying the mass and heating the same to distil off volatiles and low boiling constituents of the binder 10 and coal, and briquetting the resulting mass.

7. A process of making fuel briquettes which comprises pulverizing coal to such degree of fineness as will effect substantial mechanical separation of carbonaceous and 15 non-carbonaceous particles, separately collecting the carbonaceous and non-carbonaceous particles by flotation employing a liquid hydrocarbon oil, distilling the carbonaceous particles and oil together to separate therefrom volatile and low boiling constituents, and briquetting the carbonaceous matter and remaining high boiling constituents of the oil.

8. A process of making fuel briquettes 20 which comprises mixing pulverized coal and a liquid hydrocarbon binding material, and forming an adhesive film of high melting binding material on the coal particles by heating the mixture to drive off volatiles and low boiling constituents thereof, and finally briquetting the resulting mass.

9. A process of making fuel briquettes which comprises mixing pulverized carbonaceous matter and a liquid hydrocarbon binding material, carbonizing the carbonaceous mass and simultaneously forming a film of high melting binder on the individual particles thereof by distilling off volatiles and low boiling constituents, and finally 25 briquetting the mass.

10. In a process of making fuel briquettes the step of carbonizing pulverized carbonaceous matter in presence of a liquid hydrocarbon prior to briquetting with consequent conversion of the liquid to a high melting binding material.

11. A process of making a hard, substantially smokelessly burning fuel briquette from bituminous coal or lignite, which comprises distilling pulverized coal or lignite with a liquid hydrocarbon at such temperature that the coal or lignite is materially carbonized and the liquid hydrocarbon reduced to a high melting binding agent distributed as a thin film on the particles of

carbonized material, and finally briquetting the mass.

12. A process of making hard, free and smokelessly burning, porous fuel briquettes which comprises incorporating with pulverized coal a hydrocarbon binding material in fluid form, distilling the mixture for removal of volatiles and low boiling material from the coal and binding fluid and for the production of a thin film of high melting 70 binder on the coal particles and for the carbonization of coal particles, and finally briquetting the resulting mass under pressure sufficient to cause adhesion of the coated particles in a porous structure.

13. A process of making fuel briquettes which comprises mixing with pulverized coal a liquid hydrocarbon incapable in itself of forming a binder or of being converted to a satisfactory binding agent but 75 capable with heating of dissolving out of the coal material to form a binding agent, heating the mixture to dissolve out the binding material and subsequently to distil off the solvent, and briquetting the resulting 80 mass.

14. A fuel briquette composed of pulverulent particles of coal coated with a high melting hydrocarbon binder, the interstices of which briquette are unobstructed by the 85 binding material.

15. A fuel briquette composed of pulverized carbonaceous matter and a high melting binder disposed in a film on the particles of carbonaceous matter and in amount 100 less than could be incorporated by mechanical means to coat substantially all the particles.

16. A fuel briquette composed of pulverulent particles of carbonaceous matter and a 105 small amount of high melting hydrocarbon binding material disposed in thin films upon the particles and serving to bind the particles together into a hard, porous mass capable of burning freely and substantially 110 smokelessly and without crumbling or adhering to adjoining briquettes.

17. A fuel briquette comprising by weight 90 to 94 parts of pulverized carbonaceous matter and 10 to 6 parts of high melting 115 hydrocarbon binder disposed in thin films upon substantially all the particles and binding them together in a porous mass.

18. A fuel briquette composed of powdered coal, the particles of which are coated with a high melting hydrocarbon binder, and materially larger particles of coal cemented together by the binder covered particles of coal, the said briquette presenting a multitude of small unobstructed voids for escape of gas generated in combustion and being sufficiently hard and tough to avoid disintegration in handling and burning.

19. A briquette of the character described in claim 18, in which the binding material 120

is formed of volatiles exuded from the coal by distillation and remaining on the surface thereof.

20. A fuel briquette composed of pulverized carbonaceous material and a hydrocarbon binder having a melting point of 300° F. or over adhering intimately to the particles in a film so thin as to leave interstices between the particles substantially unobstructed.

21. A fuel briquette composed of carbonaceous matter in the form of particles which will pass through a 200-mesh screen and a high melting hydrocarbon binder in amount insufficient to obstruct interstices between the particles, the said briquette being sufficiently hard and tough to withstand transportation.

22. A fuel briquette capable of burning substantially smokelessly and without crumbling, said briquette being formed from bituminous coal or lignite and a liquid hydrocarbon, the said briquette being composed of particles of carbonaceous matter which will pass through a 200-mesh screen united by a binding material having a melting point of approximately 300° F. or higher.

23. In the manufacture of fuel briquettes the process of forming a film of high melting binding material upon particles of carbonaceous material which consists in mixing with pulverized carbonaceous material a liquid hydrocarbon, and distilling off volatiles and low boiling constituents of the mixture whereby high boiling constituents will remain as a thin film upon the particles of carbonaceous material.

24. A process of making fuel briquettes which consists in mixing pulverized coal and a liquid hydrocarbon, heating the mixture to drive off volatile and low boiling constituents, mixing the residue with granulated coal and briquetting the mass.

25. A process of making fuel briquettes which consists in mixing pulverized coal and a liquid hydrocarbon to produce a binding material, mixing the binding material with granulated coal, heating the final mixture to drive off volatile and low boiling constituents and briquetting the mass.

26. A method of uniformly mixing a relatively small amount of liquid hydrocarbon binding material with a relatively large amount of coal which consists in mixing the liquid binder with a portion of the coal in finely pulverized state, and then mixing the mixture of finely pulverized coal and binder with the remainder of the coal in granular state.

27. A process for making fuel briquettes, which comprises heating finely divided carbonaceous material, such as bituminous coal or lignite, for expulsion of low boiling volatiles therefrom and until volatiles having

melting points of approximately 300° F. appear at the surface of the particles, and briquetting the mass, the exuded volatiles serving to bind the particles together.

28. A process of making fuel briquettes, which comprises compressing masses of finely divided carbonaceous matter, such as bituminous coal or lignite, the individual particles of which are coated with a thin film of binding material being volatile matter expelled from the particles themselves prior to compression, the said film serving to bind the particles together after compression in a hard porous mass.

29. A process of making fuel briquettes, which comprises heating finely divided carbonaceous material, such as bituminous coal or lignite, for expulsion of low boiling volatiles therefrom and until volatiles having melting points of approximately 300° F. appear at the surface of the particles, intimately mixing the mass with less finely divided particles of carbonaceous material such as anthracite coal, and briquetting the mixture.

30. Mixing together finely divided carbonaceous matter such as anthracite or bituminous coal or lignite and hydrocarbon oil, distilling the mixture and collecting volatiles which come off up to approximately 650° Farenheit, and retaining the residual solid mass for use as fuel.

31. Mixing together finely divided carbonaceous matter such as bituminous coal or lignite and a hydrocarbon oil such as crude petroleum, distilling the mixture at a temperature of 650° Farenheit and upwards, and collecting the volatiles obtained from the distillation.

32. A process of preparing high volatile carbonaceous material such as bituminous coal and lignite for use as fuel and obtaining volatile constituents therefrom, which comprises extracting a portion of the lower boiling volatiles from the coal by mixing the carbonaceous material in finely divided form with a hydrocarbon oil such as crude petroleum, and distilling the mixture.

33. A process of treating high volatile coals and lignites for the preparation of smokeless fuel therefrom, which comprises distilling the coal or lignite in finely divided state and in admixture with a hydrocarbon oil for the removal of the lower boiling volatiles thereof, and separately collecting the solid residue and the expelled volatiles.

34. A briquette of the character described in claim 18, in which the binding material is composed in part of volatiles exuded from the coal by distillation and remaining upon the surface thereof and in part of the residue of a liquid hydrocarbon binding material distilled with the coal.

35. A fuel briquette comprising particles of powdered coal coated with a thin film of

high melting hydrocarbon binder admixed with and cementing together uncoated coal particles, being volatile matter exuded from the coal in distillation and remaining upon the surface thereof.

10

tough and porous.

5 36. A fuel briquette composed of distilled and undistilled coal particles and a binding

material upon the surface of the distilled

In witness whereof, I have hereunto set my hand.

HUGH H. HANSARD.